# EUROPEAN PATENT APPLICATION

(11) **EP 4 787 076 A1**
(43) Date of publication of application: **05.08.2026**
(21) Application number: 24872042.7
(22) Date of filing: 19.09.2024
(51) Int. Cl.: G03G 9/087, G03G 9/097

(54) **CRYSTALLINE-POLYESTER-CONTAINING TONER**

(30) Priority: 29.09.2023 JP 2023170757
(71) Applicant: Tomoegawa Corporation, Tokyo 104-8335 (JP)
(72) Inventor: JINNO, Yuuki, Shizuoka-shi, Shizuoka 421-0192 (JP); MORIWAKI, Naoya, Shizuoka-shi, Shizuoka 421-0192 (JP)
(74) Representative: Hoffmann Eitle
(86) International application number: PCT/JP2024/033518
(87) International publication number: WO 2025/070251

(57) **Abstract**

Provided is a toner having excellent low-temperature fixability and better heat-resistant storage stability. A toner according to an aspect contains a resin, a wax, and a pigment. The resin contains a crystalline polyester and an amorphous resin, and the crystalline polyester contains a dicarboxylic acid component having 10 to 12 carbon atoms and a diol component having 2 to 8 carbon atoms as constituent raw materials.

## Description

### Technical Field

The present invention relates to a crystalline polyester-containing toner.

### Background Art

Electrophotography is widely used as a means of an image forming method in a copier, a printer, a facsimile, or the like. General image formation by electrophotography includes: a development step of forming an electrostatic latent image by irradiating a photoconductive insulator (photoreceptor) uniformly charged using a contact charging roller or a corona charger using corona discharge with laser light, LED light, or the like, and electrostatically attaching an electrostatic charge image developing toner (hereinafter, when it is simply referred to as a toner, this has the same meaning) to the electrostatic latent image to form a toner image; a transfer step of transferring the toner image to a recording medium such as a medium to be recorded; and a fixing step of melting the transferred toner image on the recording medium by contact with a heat medium, infrared irradiation, or the like and then radiating heat to fix the toner image. In recent years, a technique enabling low-temperature fixing has been developed from a viewpoint of energy saving in the fixing step. The fact that such a toner having excellent low-temperature fixability easily causes a blocking phenomenon in which particles of the toner are aggregated due to heat generated from a machine used, heat during storage, or the like, and is inferior in heat-resistant storage stability is seen as a problem. In order to solve such a problem, for example, a toner disclosed in Patent Literature 1 is proposed as a toner capable of achieving both low-temperature fixability and heat-resistant storage stability.

### Citation List

### Patent Literature

Patent Literature 1: JP 2006-084743 A

### Summary of Invention

### Technical Problem

Patent Literature 1 discloses that a toner satisfying 10°C < (T1 - T2) < 60°C, in which T1 represents a glass transition temperature of the toner that has been heated from -20°C to 150°C at a temperature rising rate of 10°C/min before thermal melting, and T2 represents a glass transition temperature of the toner that has been heated from -20°C to 150°C at a temperature rising rate of 10°C/min, then has been cooled to -20°C at a temperature falling rate of 10°C/min, and then has been further heated at a temperature rising rate of 10°C/min after thermal melting, a toner satisfying 0 < Q2/Q1 < 2/3, in which Q1 represents an endothermic amount of a melting point peak before thermal melting, and Q2 represents an endothermic amount of a melting point peak after thermal melting, and a toner satisfying 10°C < (T1 - T2) < 60°C and 0 < Q2/Q1 < 2/3 can achieve both low-temperature fixability and heat-resistant storage stability. However, since the toner of Patent Literature 1 contains a low-softening-point resin or the like having excellent low-temperature fixability, the toner has excellent low-temperature fixability, but may be insufficient in heat-resistant storage stability.

Therefore, an object of the present invention is to provide a toner having excellent low-temperature fixability and better heat-resistant storage stability.

### Solution to Problem

In order to solve the above problems, the toner of the present disclosure contains a plurality of specific resins. That is, the present disclosed technique is as follows.

An aspect of the present disclosed technique is
a toner containing a resin, a wax, and a pigment, in which the resin contains a crystalline polyester and an amorphous resin, and the crystalline polyester contains a dicarboxylic acid component having 10 to 12 carbon atoms and a diol component having 2 to 8 carbon atoms as constituent raw materials.

The content of the crystalline polyester is preferably 0.5 to 10.0% by mass based on the mass of the resin.

The content of the crystalline polyester is preferably 2.0 to 4.0% by mass based on the mass of the resin.

The toner further contains a domain formed of the crystalline polyester and the wax, and the domain preferably has an average diameter of 75 nm or less.

A molecular weight distribution curve obtained by gel permeation chromatography (GPC) measurement of the toner includes a peak Sp having a peak top at a molecular weight (M) of 1 × 10⁵ to 1 × 10⁷, and when a value on the vertical axis at a molecular weight (M) of 1 × 10⁵ in the molecular weight distribution curve is Pb, a ratio (Pt/Pb) of a height (maximum value) Pt of the peak top of the peak Sp on the vertical axis to Pb is preferably 1.3 or more.

Note that the horizontal axis of the molecular weight distribution curve indicates a molecular weight, and the vertical axis of the molecular weight distribution curve indicates an area%.

The area% is an area% of each peak based on a total area of all peaks in a spectrum obtained with the horizontal axis as a retention time and the vertical axis as a detection intensity obtained by a differential refractive index detector in GPC measurement of the toner.

GPC measurement conditions are described below.
Temperature in column: 40°C
Eluent composition: tetrahydrofuran
Eluent flow rate: 1.0 mL/min
Standard reagent for calibration: standard polystyrene
Detector: differential refractive index detector
Detector temperature: room temperature

### Advantageous Effects of Invention

According to the present invention, by forming a toner containing a plurality of specific resins, it is possible to provide a toner having excellent low-temperature fixability and better heat-resistant storage stability.

### Brief Description of Drawings

[Fig. 1] Fig. 1 is an explanatory diagram for explaining a molecular weight distribution curve of a toner.

### Description of Embodiments

In the present disclosure, a simple compound name includes all isomers thereof.

In the present disclosure, "(meth)acrylic", "(meth)acrylic acid", and the like mean "acrylic and/or methacrylic", "acrylic acid and/or methacrylic acid", and the like.

### 1. Toner

A toner of the present disclosure preferably contains a resin, a wax, and a pigment. The resin preferably contains a crystalline polyester and an amorphous resin, and the crystalline polyester preferably contains a dicarboxylic acid component having 10 to 12 carbon atoms and a diol component having 2 to 8 carbon atoms as constituent raw materials.

A structure of a toner particle constituting the toner is not particularly limited, and examples thereof include a toner particle having a core-shell structure in which a particulate core is a uniform toner component, and a part or the whole of a surface of the core is coated with a resin layer different from the toner component.

An average particle diameter of the toner particles is not particularly limited as long as an effect of the present embodiment is not impaired, but is, for example, preferably 3 to 18 µm, more preferably 3 to 12 µm, and still more preferably 3 to 10 µm. When the average particle diameter of the toner particles is in such a range, it is relatively easy to manufacture the toner particles, and it is possible to obtain an effect of suppressing the amount of the toner particles used at the time of printing and obtaining clear printing.

Note that the average particle diameter of the toner particles is a volume average particle diameter, and can be measured using a commercially available apparatus, for example, a Coulter counter, and the volume average particle diameter means a volume 50% diameter.

The thickness of the resin layer which is a shell when the toner particle has a core-shell structure is not particularly limited, and for example, a lower limit of the thickness of the resin layer can be 10 nm or more, 15 nm or more, 20 nm or more, 30 nm or more, 40 nm or more, 50 nm or more, or 100 nm or more. An upper limit of the thickness of the resin layer can be 500 nm or less, 450 nm or less, 400 nm or less, 300 nm or less, or 200 nm or less.

As a material of the resin layer which is a shell in a case where the toner particle has a core-shell structure, for example, an amino-based resin, a urea-formaldehyde resin, a melamine resin, a benzoguanamine resin, a urea resin, a polyamide resin, an epoxy resin, a polyvinyl and polyvinylidene-based resin, an acrylic resin, a polymethyl methacrylate resin, a polyacrylonitrile resin, a polyvinyl acetate resin, a polyvinyl alcohol resin, a polyvinyl butyral resin, a polystyrene-based resin such as a polystyrene resin or a styrene-acrylic copolymer resin, a halogenated olefin resin such as polyvinyl chloride, a polyester-based resin such as a polyethylene terephthalate resin or a polybutylene terephthalate resin, a polycarbonate-based resin, a polyethylene resin, a polyvinyl fluoride resin, a polyvinylidene fluoride resin, a polytrifluoroethylene resin, a polyhexafluoropropylene resin, a copolymer of vinylidene fluoride and an acrylic monomer, a copolymer of vinylidene fluoride and vinyl fluoride, a fluoroterpolymer such as a terpolymer of tetrafluoroethylene, vinylidene fluoride, and a non-fluorinated monomer, and a silicone resin can be used.

A molecular weight distribution curve (see Fig. 1) obtained by gel permeation chromatography (GPC) measurement of the toner (containing all toner components) includes a peak Sp having a peak top in a molecular weight (M) range of 1 × 10⁵ to 1 × 10⁷, and when a value on the vertical axis at a molecular weight (M) of 1 × 10⁵ in the molecular weight distribution curve is Pb, a ratio (Pt/Pb) of a height (maximum value) Pt of the peak top of the peak Sp on the vertical axis to Pb is preferably 1.3 or more, more preferably 1.3 or more and 4.0 or less, and still preferably 1.3 or more and 3.0 or less. When Pt/Pb is in such a range, fixability and heat-resistant storage stability of the toner are favorable, and moldability is also favorable.

Note that the horizontal axis of the molecular weight distribution curve indicates a molecular weight (M), and the vertical axis of the molecular weight distribution curve indicates an area%. Here, the area% is an area% of each peak based on a total area of all peaks in a spectrum (GPC measurement result) obtained with the horizontal axis as a retention time and the vertical axis as a detection intensity obtained by a differential refractive index detector in GPC measurement of the toner.

GPC measurement conditions are described below.
Temperature in column: 40°C
Eluent composition: tetrahydrofuran
Eluent flow rate: 1.0 mL/min
Standard reagent for calibration: standard polystyrene
Detector: Differential refractive index detector
Temperature: room temperature

More specific examples of the GPC measurement are as follows.

In 10.0 ml of tetrahydrofuran (THF), 20.0 mg of the toner is dissolved, the resulting solution is centrifuged (4°C, 2000 rpm × 10 min) using a centrifuge, and a supernatant is taken out. When the toner is hardly dissolved in THF, dissolution of the toner can be promoted by heating THF. A heating temperature is not particularly limited, and can be, for example, 60°C.

The resulting supernatant is subjected to GPC measurement under the above conditions to obtain a spectrum (GPC measurement result of the toner) obtained with the horizontal axis as a retention time and the vertical axis as a detection intensity obtained by a differential refractive index detector.

Subsequently, apart from the GPC measurement of the toner, GPC measurement is performed on several kinds of standard polystyrenes having different molecular weights, and using a calibration curve prepared by creating a graph of a molecular weight (M) with respect to a retention time, the horizontal axis of the spectrum (GPC measurement result of the toner) is converted from the retention time to the molecular weight (logM). In addition, the detection intensity obtained by a differential refractive index detector, which is the vertical axis of the spectrum (GPC measurement result of the toner), is converted to an area% of each peak based on the total area of all peaks in the obtained spectrum (GPC measurement result) to create a molecular weight distribution curve.

Here, the molecular weight of the standard polystyrene used for creating the calibration curve is not particularly limited, but for example, a polystyrene having a molecular weight of 5,480,000, a polystyrene having a molecular weight of 427,000, a polystyrene having a molecular weight of 96,400, a polystyrene having a molecular weight of 16,200, and a polystyrene having a molecular weight of 2,630 can be used in combination.

A GPC device used for the GPC measurement is not particularly limited, but for example, an EXTREMA GPLC system (manufactured by JASCO Corporation) can be used. A column used for the GPC measurement is not particularly limited, but a column obtained by connecting two Shodex 806 L columns (manufactured by Showa Denko K.K.) can be used.

The toner of the present disclosure preferably further contains a domain formed of a crystalline polyester and a wax in the toner. The domain refers to a state of forming a sea-island structure in which a crystalline polyester and a wax are forming an island in a sea of an amorphous polyester.

A domain average diameter in the toner is preferably 50 nm or more, 53 nm or more, 55 nm or more, or the like, and preferably 80 nm or less, 78 nm or less, 75 nm or less, or the like. A domain average area in the toner is preferably 1,700,000 nm² or more, 1,800,000 nm² or more, 1,900,000 nm² or more, or the like, and is preferably 5,000,000 nm² or less, 2,300,000 nm² or less, 2,200,000 nm² or less, or the like. A domain average area × an average value of the number of domains per unit area is preferably 4,200 (nm²/µm²) or less.

By setting the domain average diameter and the domain average area in the toner and the domain average area × the average value of the number of domains per unit area within the above numerical ranges, exposure of the crystalline polyester, which is a material having a low melting point, and the wax to a surface is suppressed. Therefore, a glass transition point is less likely to decrease, and a toner having excellent heat-resistant storage stability can be obtained.

A method for measuring the domain average diameter and the domain average area in the toner and the average value of the number of domains per unit area will be described. First, the toner is encapsulated in a room temperature curable resin to prepare a section sample. Scanning transmission electron detector (STEM) analysis is performed on the section sample. The obtained SEM image is binarized into a crystalline portion and an amorphous portion using image analysis software. The domain average diameter, the domain average area, and the average value of the number of domains per unit area are calculated from the crystalline portion of the binarized image.

### 1-1. Resin

### 1-1-1. Crystalline polyester

The toner preferably contains a crystalline polyester. The crystalline polyester has a degree of crystallinity of 10% or more, and an endothermic peak due to melting of a crystal component is preferably clearly observed in differential scanning calorimetry (DSC).

The crystalline polyester preferably contains a dicarboxylic acid component having 10 to 12 carbon atoms and a diol component having 2 to 8 carbon atoms as constituent raw materials. That is, the crystalline polyester is preferably obtained by a reaction between a dicarboxylic acid component having 10 to 12 carbon atoms and a diol component having 2 to 8 carbon atoms.

The dicarboxylic acid component having 10 to 12 carbon atoms is not particularly limited, and examples thereof include an aliphatic dicarboxylic acid, an aromatic dicarboxylic acid, an alicyclic carboxylic acid, and derivatives thereof. As these dicarboxylic acids, either a saturated dicarboxylic acid or an unsaturated dicarboxylic acid can be used. These can be used singly or in combination of two or more thereof at any ratio.

Among these dicarboxylic acids, an aliphatic dicarboxylic acid is preferable, 1,8-octanedicarboxylic acid, 1,9-nonanedicarboxylic acid, 1,10-decanedicarboxylic acid, structural isomers of these dicarboxylic acids, and derivatives of these dicarboxylic acids are more preferable, 1,8-octanedicarboxylic acid, 1,9-nonanedicarboxylic acid, 1,10-decanedicarboxylic acid, and derivatives of these dicarboxylic acids are still more preferable, and 1,8-octanedicarboxylic acid, 1,9-nonanedicarboxylic acid, and 1,10-decanedicarboxylic acid are particularly preferable.

The diol component having 2 to 8 carbon atoms is not particularly limited, and examples thereof include: an aliphatic diol, an aromatic diol, an alicyclic diol, an aliphatic ether diol, 1,4-bis(hydroxymethyl) cyclohexane; an etherified bisphenol such as bisphenol A, hydrogenated bisphenol A, polyoxyethylenated bisphenol A, or polyoxypropylenated bisphenol A; and other dihydric alcohol monomers and derivatives thereof. As these diols, either a saturated diol or an unsaturated diol can be used. These can be used singly or in combination of two or more thereof at any ratio.

Among these diols, an aliphatic diol and an aliphatic ether diol are preferable, 1,2-ethanediol, 1,3-propanediol, 1,4-butanediol, 1,5-pentanediol, 1,6-hexanediol, 1,7-septanediol, 1,8-octanediol, neopentyl glycol, structural isomers of these diols, and derivatives of these diols are more preferable, 1,2-ethanediol, 1,3-propanediol, 1,4-butanediol, 1,5-pentanediol, 1,6-hexanediol, 1,7-septanediol, 1,8-octanediol, neopentyl glycol, and derivatives of these diols are still more preferable, and 1,2-ethanediol, 1,3-propanediol, 1,4-butanediol, 1,5-pentanediol, 1,6-hexanediol, 1,7-septanediol, 1,8-octanediol, and neopentyl glycol are particularly preferable.

A weight average molecular weight (Mw) of the crystalline polyester is preferably 10,000 to 30,000, and more preferably 10,000 to 21,000. The weight average molecular weight (Mw) of the crystalline polyester can be determined by the GPC measurement described above. When the weight average molecular weight (Mw) of the crystalline polyester is in such a range, fixability and heat-resistant storage stability of the toner are favorable, and moldability is also favorable.

The weight average molecular weight (Mw) of the crystalline polyester can be measured in a similar manner to that in the GPC measurement of the toner except that centrifugation is performed.

A melting point of the crystalline polyester is preferably 50°C or higher and lower than 100°C, more preferably 60°C or higher and lower than 90°C, and still more preferably 70°C or higher and lower than 85°C. When the melting point of the crystalline polyester is in such a range, fixability and heat-resistant storage stability of the toner are favorable, and moldability is also favorable.

The melting point of the crystalline polyester is determined using a DSC curve and defined as follows. The DSC curve is obtained at the time of temperature rise when DSC measurement is performed in accordance with ASTM D3418-82 or JIS K7121-1987. As a specific measurement method, first, about 10 mg of a sample is put in an aluminum cell, the cell is placed on a differential scanning calorimeter (trade name: SCC-6200 manufactured by Seiko Instruments Inc.), and measurement is performed while 50 ml of N₂ gas per minute is blown thereinto. Then, the temperature is raised from 20°C to 110°C at a rate of 10°C per minute, and held at 110°C for 10 minutes to remove a thermal history at a temperature equal to or lower than a glass transition temperature (Tg) region of the crystalline polyester. Next, the temperature is lowered from 110°C to 20°C at a rate of 10°C per minute, and held at 20°C for 10 minutes. Next, the temperature is raised for the second time from 20°C to 250°C at a rate of 10°C per minute, and in the DSC temperature rising curve observed at this time, a peak temperature of an endothermic peak due to melting of a crystal component is defined as a melting point.

The glass transition temperature (Tg) of the crystalline polyester is not particularly limited, but is preferably 40 to 100°C, more preferably 50 to 90°C, and still more preferably 60 to 80°C. When the glass transition temperature (Tg) of the crystalline polyester is in such a range, fusion resistance of the toner is favorable, and fixing strength and moldability of the toner are favorable.

The Tg of the crystalline polyester can be measured by the following method.

About 10 mg of a sample is put in an aluminum cell, the cell is placed on a differential scanning calorimeter (trade name: SCC-6200 manufactured by Seiko Instruments Inc.), and measurement is performed in accordance with JIS K 7121-1987 while 50 ml of N₂ gas per minute is blown thereinto. First, the temperature is raised from -20°C to 110°C at a rate of 10°C per minute, and held at 110°C for 10 minutes (the sample is left to stand at a glass transition temperature (Tg) of the sample or lower) to remove a thermal history. Next, the temperature is lowered from 110°C to -20°C at a rate of 10°C per minute, and held at -20°C for 10 minutes. Next, the temperature is raised for the second time from -20°C to 110°C at a rate of 10°C per minute, and from the DSC temperature rising curve observed at this time, a midpoint glass transition temperature (Tmg) described in 9.3 of the above JIS K 7121-1987 is determined, and this temperature is defined as Tg of the present embodiment.

The degree of crystallinity of the crystalline polyester is not particularly limited as long as it is 10% or more, but is preferably 20 to 70% and more preferably 30 to 80% from a viewpoint of improvement of fixing characteristics, moldability, and the like. The degree of crystallinity can be increased by molding conditions or by using a crystal nucleating agent. The degree of crystallinity can be determined by an X-ray diffraction method.

### 1-1-2. Amorphous resin

As the amorphous resin, a known resin for a toner can be used, and is not particularly limited, but examples thereof include: a polyester; a styrene-(meth)acrylic acid-based copolymer resin; a styrene-based resin such as polystyrene, poly-α-methylstyrene, polychlorostyrene, a styrene-propylene copolymer, a styrene-butadiene copolymer, a styrene-vinyl chloride copolymer, a styrene-vinyl acetate copolymer, a styrene-maleic acid copolymer, or a styrene-acrylonitrile-acrylic acid ester copolymer; a (meth)acrylic acid-based resin; a rosin-modified maleic acid resin; an olefin-based resin such as polyethylene or polypropylene; a polycarbonate; a polyether-based resin; a (modified) polyphenylene ether; a vinyl-based resin such as polyvinyl chloride or polyvinylidene chloride; a urethane-based resin; a phenol resin; an epoxy-based resin; a polyphenylene oxide-based resin; a terpene phenol resin; a polylactic acid resin; a hydrogenated rosin; a cyclized rubber; an ionomer resin; a silicone resin; a ketone resin; a xylene resin; an ABS resin; a cycloolefin-based copolymer resin; a petroleum-based resin; and a hydrogenated petroleum-based resin. These amorphous resins can be used singly or in combination of two or more thereof at any ratio. Among these, a polyester and a styrene-(meth)acrylic acid-based copolymer resin are preferable from a viewpoint that requirements of image quality characteristics, durability, productivity, and the like of the toner can be satisfied in a well-balanced manner.

A weight average molecular weight (Mw) of the amorphous resin is preferably 5,000 to 60,000, and more preferably 8,000 to 40,000. The weight average molecular weight (Mw) of the amorphous resin can be determined by the GPC measurement described above. In addition, in the molecular weight distribution curve of the amorphous resin obtained by the GPC measurement, the molecular weight (M) of the amorphous resin preferably has a peak top in a range of 1 × 10⁵ to 1 × 10⁷. In this case, it is easy to adjust the peak top of the peak Sp in the molecular weight distribution curve of the toner so as to be in a molecular weight (M) range of 1 × 10⁵ to 1 × 10⁷.

A melting point of the amorphous resin is preferably 50°C or higher and lower than 180°C, more preferably 60°C or higher and lower than 170°C, and still more preferably 70°C or higher and lower than 160°C. When the melting point of the amorphous resin is in such a range, fixability and fusion resistance are favorable, and moldability is also favorable. The melting point of the amorphous resin can be determined in a similar manner to that for the melting point of the crystalline polyester.

A glass transition temperature (Tg) of the amorphous resin is preferably 30 to 80°C, and more preferably 40 to 70°C. When the glass transition temperature (Tg) of the amorphous resin is in such a range, fusion resistance and heat storage stability are favorable, and fixing strength is also excellent. The glass transition temperature (Tg) of the amorphous resin can be determined in a similar manner to that for the glass transition temperature (Tg) of the crystalline polyester.

### 1-2. Wax

The toner may contain a wax. The wax is not particularly limited as long as it has favorable dispersibility or the like with the crystalline polyester and the amorphous resin, and examples thereof include: a polyolefin-based wax such as a polyethylene wax, a polypropylene wax, or a modified polyethylene wax; a synthetic wax such as a Fischer-Tropsch wax or a polyester-based synthetic wax; a petroleum-based wax such as a paraffin wax or a microcrystalline wax; an animal wax such as a beeswax or a spermaceti wax; a plant wax such as a carnauba wax, a candelilla wax, or a rice wax; a hardened oil such as a hardened castor oil; and a mineral wax such as a montan wax, ozokerite, or ceresin. These waxes can be used singly or in combination of two or more thereof at any ratio. Among these waxes, an animal wax and a plant wax having a low melting point are preferable from a viewpoint of low-temperature fixability, but a rice wax and a carnauba wax having a melting point that is not too low are more preferably used from a viewpoint of heat-resistant storage stability of the toner, and a rice wax is still more preferable from a viewpoint of offset resistance.

A melting point of the wax is preferably 50 to 120°C, more preferably 50 to 100°C, and still more preferably 50 to 85°C. When the melting point of the wax is in such a range, fusion resistance and heat storage stability of the toner are favorable, and fixability and fixing strength are also favorable.

The melting point of the wax is measured in accordance with ASTM D3418-82 as follows.

About 10 mg of a sample is weighed and put in an aluminum cell, the cell is placed on a differential scanning calorimeter (DSC) (trade name: SCC-6200 manufactured by Seiko Instruments Inc.), and 50 ml of N₂ gas per minute is blown thereinto. Then, the temperature is raised from 20°C to 200°C at a rate of 10°C per minute, held at 200°C for 10 minutes, then lowered from 200°C to 20°C at a rate of 10°C per minute, and then raised for the second time under the above conditions, and the temperature at a top of a maximum endothermic peak at this time is defined as the melting point.

### 1-3. Pigment

The toner preferably contains a pigment. Examples of a pigment for a black toner include a pigment for black, and examples of a pigment for a color toner include a pigment for magenta, a pigment for cyan, a pigment for yellow, and a toner for full color.

Examples of the pigment for black include carbon black, iron oxide, magnetite, and ferrite, and the pigment for black preferably contains carbon black. The number average particle diameter, oil absorption amount, pH, and the like of carbon black are not particularly limited. Examples of a commercially available product include REGAL 400, REGAL 660, REGAL 330, REGAL 300, REGAL SRF-S, STERLING SO, STERLING V, STERLING NS, and STERLING R manufactured by Cabot Corporation; RAVEN H20, RAVEN MT-P, RAVEN410, RAVEN420, RAVEN430, RAVEN450, RAVEN500, RAVEN760, RAVEN780, RAVEN1000, RAVEN1035, RAVEN1060, and RAVEN1080 manufactured by Columbian Carbon Japan Co., Ltd.; and #5B, #10B, #40, #2400B, and MA-100 manufactured by Mitsubishi Chemical Corporation. These carbon blacks can be used singly or in combination of two or more thereof at any ratio.

Examples of the pigment for magenta include C.I. Pigment Red 1, 2, 3, 4, 5, 6, 7, 8, 9, 10, 11, 12, 13, 14, 15, 16, 17, 18, 19, 21, 22, 23, 30, 31, 32, 37, 38, 39, 40, 41, 48, 49, 50,51, 52, 53, 54, 55, 57, 58, 60, 63, 64, 68, 81, 83, 87, 88, 89, 90, 112, 114, 122, 123, 163, 202, 206, 207, 209, and 269; C.I. Pigment Violet 19; and C.I. Bat Red 1, 2, 10, 13, 15, 23, 29, and 35. These pigments for magenta can be used singly or in combination of two or more thereof at any ratio.

Examples of the pigment for cyan include C.I. Pigment Blue 2, 3, 15, 16, and 17; C.I. Bat Blue 6; and C.I. Acid Blue 45. These pigments for cyan can be used singly or in combination of two or more thereof at any ratio.

Examples of the pigment for yellow include C.I. Pigment Yellow 1, 2, 3, 4, 5, 6, 7, 10, 11, 12, 13, 14, 15, 16, 17, 23, 65, 73, 74, 83, 93, 94, 97, 155, and 180. These pigments for yellow can be used singly or in combination of two or more thereof at any ratio.

As the color pigment of the toner for full color, it is preferable to use C.I. Pigment Red 57 or 122 as a pigment for magenta, C.I. Pigment Blue 15 as a pigment for cyan, and C.I. Pigment Yellow 17, 93, 155, or 180 as the pigment for yellow from a viewpoint of color mixing properties and color reproducibility.

### 1-4. Other components

The toner can contain various additives as necessary. Examples of other components include a charge control agent, a magnetic powder, a crystal nucleating agent, external fine particles, a stabilizer (for example, an ultraviolet absorber, an antioxidant, or a heat stabilizer), a flame retardant, an antifogging agent, a dispersant, a plasticizer (a phthalate, a fatty acid-based plasticizer, a phosphoric acid-based plasticizer, or the like), a polymeric antistatic agent, a low molecular antistatic agent, a compatibilizer, a conductive agent, a filler, and a fluidity improver.

### 1-4-1. Charge control agent

The electrostatic charge image developing toner of the present embodiment may contain a charge control agent as necessary.

Examples of a positively chargeable charge control agent include: a product modified by nigrosine, a fatty acid metal salt thereof, or the like; a quaternary ammonium salts such as tributylbenzylammonium-1-hydroxy-4-naphthosulfonate or tetrabutylammonium tetrafluoroborate; a diorganotin oxide such as dibutyltin oxide, dioctyltin oxide, or dicyclohexyltin oxide; a diorganotin borate such as dibutyltin borate, dioctyltin borate, or dicyclohexyltin borate; a pyridium salt, an azine, a triphenylmethane-based compound, and a low molecular weight polymer having a cationic functional group. These positively chargeable charge control agents may be used singly or in combination of two or more thereof. Among these positively chargeable charge control agents, a nigrosine-based compound and a quaternary ammonium salt are preferably used.

Examples of a negatively chargeable charge control agent include an organometallic compound such as an acetylacetone metal complex, a monoazo metal complex, or a naphthoic acid or salicylic acid-based metal complex or metal salt, a chelate compound, and a low molecular weight polymer having an anionic functional group. These negatively chargeable charge control agents can be used singly or in combination of two or more thereof at any ratio. Among these negatively chargeable charge control agents, a salicylic acid-based metal complex and a monoazo metal complex are preferably used.

### 2. Method for manufacturing toner

### 2-1. Method for manufacturing toner

A method for manufacturing the toner of the present embodiment is not particularly limited, but examples thereof include a method in which a crystalline polyester, an amorphous resin, a wax, and a pigment are mixed and kneaded, and the obtained resin composition is pulverized and classified.

As a mixing method, a known method can be used, and examples thereof include a method for obtaining a mixture using a mixing device such as a double cone mixer, a V-type mixer, a drum-type mixer, a super mixer, a Henschel mixer, or a Nauta mixer.

The obtained mixture is kneaded to uniformly disperse the pigment and any components in the resin to obtain a kneaded product. As a kneading method, a batch type (for example, a pressure kneader or a Banbury mixer) or a continuous hot-melt kneader can be used, but a uniaxial or biaxial continuous extruder is preferable from a viewpoint of superiority such as continuous production.

As a more specific hot-melt kneading method, for example, the mixture is hot-melt kneaded by a twin-screw extruder and extruded from a spinneret (die) at a distal end of the twin-screw extruder to obtain a kneaded product. A kneading temperature of the twin-screw extruder is usually about 70 to 250°C, preferably about 70 to 200°C, and more preferably about 90 to 200°C.

In order to sufficiently melt the crystalline polyester to enhance moldability, the kneading temperature is preferably a temperature equal to or higher than a temperature 20°C lower than the melting point of the crystalline polyester and equal to or lower than a temperature 30°C higher than the melting point of the crystalline polyester.

Examples of a pulverization method include a method in which coarse pulverization is first performed with a crusher, a hammer mill, a feather mill, or the like, and subsequently fine pulverization is performed with a jet mill, a counter jet mill, a highspeed rotor rotary mill, or the like to perform pulverization stepwise up to a predetermined toner particle size.

Examples of a classification method include a method in which the toner is classified by an inertial classification type Elbow jet, a centrifugal classification type Microplex, a DS separator, a dry air flow classifier, or the like to obtain a classified toner having a predetermined volume average particle diameter.

The inorganic fine particles and the resin fine powder may be attached to a surface of the toner by performing stirring using a stirrer such as a turbine type stirrer, a Henschel mixer, or a super mixer.

The content of the crystalline polyester in the toner is preferably 0.1 to 20.0% by mass, more preferably 0.5 to 15.0% by mass, and still more preferably 1.0 to 10.0% by mass based on the total mass of the toner. In addition, the content of the crystalline polyester in the toner is preferably 0.5 to 10.0% by mass, more preferably 1.0 to 5.0% by mass, still more preferably 2.0 to 4.0% by mass, and further still more preferably 2.0 to 3.0% by mass based on the mass of the resin (the sum of the mass of the crystalline polyester and the mass of the amorphous resin). When the content of the crystalline polyester is in such a range, fixability, resin strength, and fusion resistance are better, and moldability of the toner is also better. Furthermore, since mechanical strength of the resin is moderate, processability such as toner pulverization is also favorable, and various characteristics such as image quality characteristics and charging characteristics can be made favorable.

The content of the amorphous resin in the toner is preferably 50 to 90% by mass, more preferably 55 to 85% by mass, and still more preferably 60 to 80% by mass based on the total mass of the toner. By adjusting the content of the amorphous resin, the position (molecular weight (M)) of the peak top of the peak Sp, the height (Pt) of the peak top of the peak Sp, and the height (Pb) at a molecular weight (M) of 1 × 10⁵ in the molecular weight distribution curve of the toner can be easily adjusted. When the content of the amorphous resin is in such a range, fixability, resin strength, and fusion resistance are better, and moldability of the toner is also better. Furthermore, since mechanical strength of the resin is moderate, processability such as toner pulverization is also favorable, and various characteristics such as image quality characteristics and charging characteristics can be made favorable.

The content of the pigment in the toner is preferably 0.1 to 30.0% by mass, more preferably 1.0 to 25.0% by mass, and still more preferably 5.0 to 20.0% by mass based on the total amount of the toner. When the content of the pigment is in such a range, image density, image quality, and moldability of the toner are better.

The content of the wax in the toner is preferably 0.1 to 30.0% by mass, more preferably 1.0 to 25.0% by mass, and still more preferably 5.0 to 20.0% by mass based on the total mass of the toner. By adjusting the content of the wax, the height (Pb) at a molecular weight (M) of 1 × 10⁵ in the molecular weight distribution curve of the toner can be adjusted. When the content of the wax is in such a range, fixability and fusion resistance are better, and moldability of the toner is also better. Furthermore, it is possible to obtain a toner in which fusion resistance, heat storage stability, and the like are synergistically improved remarkably.

The content when the charge control agent is used is preferably 0.1 to 5.0% by mass, more preferably 0.5 to 4.0% by mass, and still more preferably 1.0 to 4.0% by mass based on the total mass of the toner.

### 2-2. Method for forming coating resin (shell)

A method for forming a coating resin that coats a part or the whole of a surface of a core particle using a toner particle obtained by the above-described manufacturing method or the like as the core particle will be described. As a coating method with the coating resin, for example, coating can be performed with the coating resin by a known method such as a brush coating method, a drying method, a spray drying method using a fluidized bed, a rotary drying method, or an immersion drying method using a universal stirrer.

### 3. Applications of toner

The above-described toner of the present disclosure has excellent fixability and heat-resistant storage stability, and thus can be suitably used in various image forming apparatuses.

### Examples

### <Preparation of toner>

### (Preparation of crystalline polyester)

In a reaction tank equipped with a cooling tube, a heating and cooling apparatus, a thermometer, a stirrer, and a nitrogen introduction tube, 50.0 mol% of each combination of dicarboxylic acid and diol in each crystalline polyester illustrated in Table 1 and 1.5 parts of titanium dihydroxybis(triethanolaminate) as a condensation catalyst were put, and the mixture was caused to react at 180°C under a nitrogen gas flow for eight hours while generated water was distilled off. The dicarboxylic acid and the diol used as raw materials are described below.

Subsequently, while the temperature was gradually raised to 220°C, the reaction was caused for four hours under a nitrogen gas flow while generated water was distilled off, and the reaction was further caused under a reduced pressure of 0.5 to 10.0 kPa to obtain a desired crystalline polyester.

### (Raw materials)

- Dicarboxylic acid component
   Dicarboxylic acid 1: 1,10 decanedicarboxylic acid (C₁₂H₂₂O₄)
   Dicarboxylic acid 2: 1,7-heptane dicarboxylic acid (C₉H₁₆O₄)
   Dicarboxylic acid 3: 1,11 undecanedicarboxylic acid (C₁₃H₂₄O₄)
   Dicarboxylic acid 4: 1,8-octanedicarboxylic acid (C₁₀H₁₈O₄)
   Dicarboxylic acid 5: 1,9-nonanedicarboxylic acid (C₁₁H₂₀O₄)
- Diol component
   Diol 1: 1,6-hexanediol (C₆H₁₄O₂)
   Diol 2: methanediol (CH₄O₂)
   Diol 3: 1,9-nonanediol (C₉H₂₀O₂)
   Diol 4: 1,2-ethanediol (C₂H₆O₂)
   Diol 5: 1,3-propanediol (C₃H₈O₂)

### (Amorphous resin)

A polyester 1 is a polyester resin containing terephthalic acid and trimellitic acid as a polycarboxylic acid component, containing bisphenol A as a diol component, and having a softening point of 145°C, an acid value of 22.0 mgKOH/g, a weight average molecular weight (Mw) of 28,000, and a Tg (shoulder) of 60°C.

A polyester 2 is a polyester resin containing terephthalic acid as a polycarboxylic acid component, containing bisphenol A as a diol component, and having a softening point of 95°C, an acid value of 22.0 mgKOH/g, a weight average molecular weight (Mw) of 9,400, and a Tg (shoulder) of 52°C.

### (Method for manufacturing toner)

The crystalline polyester and the amorphous resin obtained by the above method, a wax, a pigment, and a charge control agent were weighed so as to be parts by mass presented in Table 1, and the following components were uniformly mixed for two minutes under a condition of 1500 rpm using a Henschel mixer (20 L Henschel mixer manufactured by Mitsui Mining Co., Ltd.) (mixing step). Thereafter, the obtained mixture was melt-mixed under conditions of a kneading temperature of 70 to 180°C, a rotation speed of 150 rpm, and a discharge amount of 3.5 kg/hr using a twin-screw extruder (PCM-30 manufactured by Ikegai Corporation) to obtain a plate-shaped resin composition.

Next, the cooled kneaded product was coarsely pulverized with a hammer mill and finely pulverized with a jet mill (trade name: "200APG" manufactured by Hosokawa Micron Corporation). Then, classification was performed with a dry air flow classifier (trade name: "100ATP" manufactured by Hosokawa Micron Corporation) to obtain classified toners of Examples and Comparative Examples having an average particle diameter of 6 to 8 µm.

### (Raw materials)

Wax: rice wax SS-1 (manufactured by Boso oil and fat Co., Ltd., melting point: 77 to 86°C)
Pigment: carbon black (ELFTEX430 manufactured by CABOT Corporation)
Charge control agent: T-77 (manufactured by Hodogaya Chemical Co., Ltd.)

### (Method for analyzing GPC. Particularly, method for creating molecular weight distribution curve)

In 10.0 ml of tetrahydrofuran (THF), 20.0 mg of the toner is dissolved, the resulting solution is centrifuged (4°C, 2000 rpm × 10 min) using a centrifuge, and a supernatant is taken out. The resulting supernatant was subjected to the GPC measurement under the following conditions to obtain a spectrum (GPC measurement result of the toner) obtained with the horizontal axis as a retention time and the vertical axis as a detection intensity obtained by a differential refractive index detector.

Subsequently, apart from the GPC measurement of the toner, GPC measurement was performed on several kinds of standard polystyrenes having different molecular weights, and using a calibration curve prepared by creating a graph of the molecular weight (M) with respect to the retention time, the horizontal axis of the spectrum (GPC measurement result of the toner) was converted from the retention time to the molecular weight (logM). In addition, the detection intensity obtained by a differential refractive index detector, which is the vertical axis of the spectrum (GPC measurement result of the toner), was converted to an area% of each peak based on the total area of all peaks in the obtained spectrum (GPC measurement result) to create a molecular weight distribution curve.

Here, as the molecular weight of the standard polystyrene used for creating the calibration curve, a polystyrene having a molecular weight of 5,480,000, a polystyrene having a molecular weight of 427,000, a polystyrene having a molecular weight of 96,400, a polystyrene having a molecular weight of 16,200, and a polystyrene having a molecular weight of 2,630 were used in combination. Pt/Pb was calculated from the obtained molecular weight distribution curve.

### •GPC measurement conditions

GPC device: EXTREMA GPLC system (manufactured by JASCO Corporation)
Column: Two Shodex 806L columns (manufactured by Showa Denko K.K.) were connected and used.
Temperature in column: 40°C
Eluent composition: tetrahydrofuran
Eluent flow rate: 1.0 mL/min
Standard reagent for calibration: standard polystyrene
Detector: differential refractive index detector
Detector temperature: room temperature

### (Method for measuring domain average diameter and domain average area)

Each of the toners obtained in Examples and Comparative Examples was encapsulated in a room temperature curing resin and cured over about three days. A section sample was prepared by an ultramicrotome EM UC6 (manufactured by Leica). The section sample was subjected to gas phase electron staining with ruthenium tetroxide (3 hr) and then observed with a scanning transmission electron detector (STEM) (JSM-7001F manufactured by JEOL Ltd.). The obtained STEM image was binarized into a crystalline portion and an amorphous portion using image analysis software (Winroof 2003).

### •STEM measurement conditions

Acceleration voltage: 30 kV
Degree of vacuum: high vacuum
Analysis magnification: ×30,000
Image detector: scanning transmission electron detector (BF mode)
Sample tilt: 0°

Absolute maximum lengths of the crystalline portions of the binarized image were measured, and an average value thereof was defined as a domain average diameter. A domain average area was calculated from a circle area formula (πr²) assuming the average diameter as a circle equivalent diameter r.

### (Evaluation)

### •Low-temperature fixability

Each of the toners obtained in Examples and Comparative Examples was used as a measurement target, and an unfixed image was photographed with a commercially available copier (LaserJet MFP M436n manufactured by HP).

A fixing machine in which a heat fixing roll whose surface layer is formed of a fluororesin and a pressure fixing roll whose surface layer is formed of a silicone rubber rotate in pairs was adjusted so as to have a roll pressure of 1 Kg/cm² and a roll speed of 150 rpm, and a surface temperature of the heat fixing roll was changed to 90 to 120°C to fix a toner image on a transfer sheet having the unfixed image at each surface temperature. Fixability was evaluated from a generation temperature of low-temperature offset of the obtained fixed image.

Evaluation criteria were as follows. Results thereof are presented in Table 1.
A: Low-temperature offset occurred below 100°C
B: Low-temperature offset occurred at 100°C or higher and below 110°C
C: Low-temperature offset occurred at 110°C or higher

### •Heat-resistant storage stability

Into a poly container having a volume of 200 mL, 10 g of each of the toners obtained in Examples and Comparative Examples was put, left to stand still in a thermo-hygrostat ("PR-3J" manufactured by ESPEC CORPORATION) set at a temperature of 50°C/humidity of 80% for 48 hours, and taken out. Next, three types of sieves with a mesh size of 150 µm, a mesh size of 75 µm, and a mesh size of 45 µm were sequentially attached to a powder tester (PT-S manufactured by Hosokawa Micron Corporation), and then 2 g of the toner was put on the sieve with a mesh size of 150 µm. A vibration amplitude was adjusted to 1.0 mm with a knob in a powder tester main body, the toner was sieved under a condition of a time of 10 seconds, the weight of the toner remaining on the sieve was measured, and a, b, c and an aggregation degree were calculated from the following formulas. Results thereof are presented in Table 1. $Aggregation degree \left(%\right) = a + b + c$ $a = \left(weight of residual toner on sieve with mesh size of 150 μm/2\right) \times 100$ $b = \left(weight of residual toner on sieve with mesh size of 75 μm/2\right) \times 100 \times \left(3/5\right)$ $c = \left(weight of residual toner on sieve with mesh size of 45 μm/2\right) \times 100 \times \left(1/5\right)$

Evaluation criteria were as follows.
A: Aggregation degree is 75% or more and less than 80%
B: Aggregation degree is 80% or more and less than 85%
C: Aggregation degree is 85% or more

### •Overall evaluation

Overall evaluation of the toners of Examples and Comparative Examples was performed according to the following evaluation criteria. Results thereof are presented in Table 1.
A: Both low-temperature fixability evaluation and heat-resistant storage stability evaluation are A.
B: One of low-temperature fixability evaluation and heat-resistant storage stability evaluation is A, and the other is B.
C: Both low-temperature fixability evaluation and heat-resistant storage stability evaluation are B.
D: Either low-temperature fixability evaluation or heat-resistant storage stability evaluation is C.

### Cross-Reference to Related Applications

The present application claims priority based on Japanese Patent Application No. 2023-170757 filed with the Japan Patent Office on September 29, 2023, the entire disclosure of which is entirely incorporated herein by reference.

## Claims

1. A toner comprising: a resin; a wax; and a pigment, wherein
the resin contains a crystalline polyester and an amorphous resin, and
the crystalline polyester contains a dicarboxylic acid component having 10 to 12 carbon atoms and a diol component having 2 to 8 carbon atoms as constituent raw materials.

2. The toner according to claim 1, wherein a content of the crystalline polyester is 0.5 to 10.0% by mass based on a mass of the resin.

3. The toner according to claim 1, wherein a content of the crystalline polyester is 2.0 to 4.0% by mass based on a mass of the resin.

4. The toner according to claim 1, further comprising a domain formed of the crystalline polyester and the wax, wherein
the domain has an average diameter of 75 nm or less.

5. The toner according to any one of claims 1 to 4, wherein
a molecular weight distribution curve obtained by gel permeation chromatography (GPC) measurement of the toner includes a peak Sp having a peak top in a molecular weight (M) range of 1 × 10⁵ to 1 × 10⁷,
when a value on a vertical axis at a molecular weight (M) of 1 × 10⁵ in the molecular weight distribution curve is Pb, a ratio (Pt/Pb) of a height (maximum value) Pt of the peak top of the peak Sp on the vertical axis to Pb is 1.3 or more,
a horizontal axis of the molecular weight distribution curve is the molecular weight (M), and the vertical axis of the molecular weight distribution curve is an area%,
the area% is an area% of each peak based on a total area of all peaks in a spectrum obtained with a horizontal axis as a retention time and a vertical axis as a detection intensity by a differential refractive index detector in GPC measurement of the toner, and
GPC measurement conditions are described below:
Temperature in column: 40°C
Eluent composition: tetrahydrofuran
Eluent flow rate: 1.0 mL/min
Standard reagent for calibration: standard polystyrene
Detector: differential refractive index detector
Detector temperature: room temperature.
